

Patented Jan. 16, 1923.

1,442,243

# UNITED STATES PATENT OFFICE.

GEORGE A. AVERY AND FREDERICK BAMBLETT, OF DETROIT, MICHIGAN.

PROCESS FOR CLEANING SCALE FROM METALS.

No Drawing.

Application filed March 23, 1922. Serial No. 546,169.

To all whom it may concern:

Be it known that we, GEORGE A. AVERY and FREDERICK BAMBLETT, citizens of the United States, residing at Detroit, in the county of Wayne and State of Michigan, have invented certain new and useful Improvements in Processes for Cleaning Scale from Metals; of which the following is a specification.

10 This invention relates to a process for cleaning scale from metals, and more particularly to a method of removing scale from hardened gears.

15 At the present time, scale is removed from hardened gears by manual labor, and by the use of wire brushes and polishing lathes. Both of these processes are costly operations, due to the labor involved and the number of brushes destroyed.

20 In the present invention, we first remove all oil and other foreign matter from the surface of the gear or other metal by treating it with a cleaning compound in a reverse current, employing a metal tank, such

25 as an iron tank, as the negative electrode. The metal is then thoroughly rinsed in water and placed in a solution of a mineral acid employing a reverse or direct current with a nickel or carbon anode as the negative electrode. This treatment will remove the most stubborn fire or oil scale in from five to ten minutes without attacking the metal in any way. The metal is then rinsed in water and dried by immersing it in a hot solution of soda which will remove all acid from the pores of the metal.

30 In a typical embodiment of the invention, the gears or other metal to be cleaned are first treated with a fairly strong solution of a metal cleaner in a reverse or direct current, using preferably from three to six volts. As stated, other metal cleaners may be employed, but it is essential that the surface of the metal be properly cleaned in order that the next step of the process may be properly carried out. As stated, the first step of the process is performed in a tank formed of a metal that is a fairly good conductor of electricity, such as an iron tank, and the tank is employed as the negative or positive electrode. The metal to be cleaned is connected to the lead wire and made the positive or negative pole during this treatment, which is carried on for a sufficient

length of time to remove all oil and other foreign matter from the surface of the metal.

35 The metal is then rinsed in water to place it in proper condition for the second step in which the scale is removed. In performing the second step of the process, the cleansed metal is placed in a solution of a mineral acid and we preferably employ a 10 per cent solution of hydrochloric and sulfuric acids in equal portions. A reverse 40 or direct current from four to six volts, with not less than two-hundred amperes is employed in this step, and a nickel or carbon electrode is used as the anode. The metal may be subjected to this treatment 45 for from five to ten minutes which will remove the most stubborn fire or oil scale, without attacking the metal in any way. It is then rinsed in water and dried by immersing it in a hot solution of an alkali, 50 such as a soda solution which will remove the acid from the pores of the metal.

55 It will be apparent to those skilled in the art that the use of this process eliminates a great deal of labor now necessary in cleaning metals and is also advantageous in that it saves the cost of the large number of wire brushes worn out or destroyed in cleaning metals according to the present process.

60 While we have described in detail, the preferred practice of our process, it is to be understood that the details of procedure, and proportion of ingredients may be widely varied, and that known chemical equivalents may be employed in place of the materials mentioned, without departing from the spirit of the invention or the scope of the subjoined claims.

65 Having thus described our invention, we claim:

70 1. The process of removing scale from metal which comprises subjecting the metal to an electric current in a solution of a cleaning composition to remove oil and other foreign matter from the surface of the metal, and then subjecting it to an electric current in a solution of a mineral acid.

75 2. The process of removing scale from metal which comprises subjecting the metal to an electric current in a solution of a cleaning composition to remove oil and other foreign matter from the surface of the metal,

then subjecting it to an electric current in a solution of a mineral acid, and then rinsing it in a soda solution.

3. The process of removing scale from metal which comprises subjecting the metal to an electric current in a solution of a cleaning composition, and then subjecting it to an electric current in a solution of hydrochloric and sulfuric acid.

10 4. The process of removing scale from metal which comprises subjecting the metal to an electric current in a solution of a cleaning composition, then subjecting it to an electric current in a solution of hydrochloric and sulfuric acid, and then rinsing it in a soda solution.

15 5. The process of cleaning metal which consists in subjecting it to an electric current in a solution of a cleaning composition to

20 remove oil from the surface of the metal, rinsing it in water, then subjecting it to an

electric current in a solution of a mineral acid, and then rinsing it in a soda solution.

6. The process of cleaning metal which comprises subjecting it to an electric current 25 of from 3 to 6 volts in a solution of a cleaning composition to remove oil from the surface of the metal, rinsing it in water, and then subjecting it to an electric current of from 4 to 6 volts, and not less than 200 30 amperes, in a solution of hydrochloric and sulfuric acid of substantially 10 per cent strength for a period of from five to ten minutes, and then rinsing it in a hot solution of soda.

35 In testimony whereof we affix our signatures in presence of two witnesses.

GEORGE A. AVERY.  
FREDERICK BAMBLETT.

Witnesses:

HARRY I. LEIBSON,  
A. E. SCHWAHN.